

1

2,907,624

## VAT DYE PRINTING

Arthur K. Saville, Wilmington, Del., assignor to E. I. du Pont de Nemours and Company, Wilmington, Del., a corporation of Delaware

No Drawing. Application August 5, 1957  
Serial No. 676,429

7 Claims. (Cl. 8—70)

This invention relates to vat dye printing, and more particularly to an improved process for the application of vat dyes to textile materials by printing processes in which the vat color is applied to the fabric in the form of a dispersion in a water-in-oil emulsion. This is a continuation-in-part of my co-pending application Serial No. 609,347, filed September 12, 1956 (now abandoned).

In the usual methods of printing textile materials with vat dyes, the vat color is dispersed in an aqueous printing paste, together with water-soluble thickeners, in which paste is also incorporated the reducing agent and alkali usually in the form of an alkali metal sulfoxylate and an alkali metal carbonate. On the passing of the textile printed with this paste into an air-free steam atmosphere, the color is converted to the leuco form and fixed into the cellulose fibers, after which the dye is reoxidized on the fiber and the goods washed to free it from the carrier and decomposition products of the reducing agent and alkali.

Alternatively, the aqueous suspension of the dye paste together with a thickener may be printed on the textile materials, and, after drying, these materials are passed rapidly through a chemical bath consisting of caustic alkali and sodium hydrosulfite directly into an air-free steamer where the dye is reduced and fixed in the fiber and then reoxidized in the usual manner.

To obviate the use of the more expensive vat dyes, methods of printing textile materials have been devised wherein a color in pigment form is dispersed in non-aqueous vehicles containing heat convertible resins, so that after printing these inks on textile materials and heating, the color is fixed to the fibers by the bonding action of the resins employed. This type of print, while having reasonable fastness to washing in pastel and light shades, suffers from severe loss of color value when printed in medium and heavy shades and subjected to washing. This type of print is particularly deficient when subjected alternatively to light exposure and washing, due to degradation of the bonding resin under these conditions. In these prints it is obvious that the color itself is not made an integral part of the textile material.

It is an object of the present invention to provide a new and improved process for printing textile materials with vat dyes in which high color value can be obtained from the vat dye which itself is reduced and attached to the fiber in the same manner as when the dye is fixed by conventional vat printing procedures. A more specific object of the invention is to provide a process for the application of vat dyes in which the vat dye is suspended in the water phase of a water-in-oil emulsion containing a temporary bonding agent which is applied to the textile materials by printing rolls having shallow intaglio engravings, and which after drying is impregnated with a chemical reducing agent comprising an alkali metal hydroxide and sodium hydrosulfite which permeates or even dissolves the resin and reduces the color whereby it is

2

fixed to the fiber in the same manner as when the vat dye is applied in the conventional printing or dyeing processes. A further object of the invention is to provide a method whereby vat colors can be printed to give sharp prints and faithful reproduction of the engraved designs at high speeds on the conventional textile printing machine, and to give excellent smoothness in the blotch areas of the print with a substantial reduction in the cost of printing vat dyes. It is a further object of the invention to produce stable textile printing compositions and concentrates which can be used as such or diluted to printing viscosities, consisting of water-in-oil emulsions in which the vat dye pigment is present in the aqueous phase.

According to the present invention, an aqueous vat dye paste of the type normally employed in printing or dyeing processes and containing a small amount of a dispersing agent, is emulsified into a water-in-oil emulsion previously formed by adding water to a water-immiscible hydrocarbon solvent which contains small amounts of a resin dissolved and/or colloidally dispersed therein. This vat dye printing paste is then applied to the textile material from the conventional textile printing equipment and conventional shallow engraved intaglio rolls which may be run at higher speeds than when employing the aqueous thickened vat dye pastes. After printing on the textile material, the prints are dried by conventional methods. Subsequently, the prints are impregnated in any conventional type of dye pad with a solution of caustic alkali and sodium hydrosulfite which may contain a wetting agent (and, if desired, a thickening agent), and then led immediately into an air-free steam atmosphere at a temperature between 212° F. and 290° F. for periods of from 7 to 30 seconds. The printed cloth is then oxidized and soaped by conventional methods, whereby the dye is converted back to the oxidized form and fixed in the fibers. During the soaping and scouring treatment, the resin which has been permeated or solubilized by the action of the caustic alkali and hydrosulfite is at least in part and usually substantially removed from the fabric.

The prints thus obtained are sharp in outline, smooth, and outstanding in strength and brightness, and at least as fast to light, washing and crocking as prints of the same dyes made by conventional vat dye procedure. In many cases the apparent strength of the prints obtained is double that obtained by printing the same color by conventional means.

This process is very versatile in that it may be employed in conjunction with the printing of the same fabrics with other types of dyes, either in an aqueous system or in an oil-in-water system, when colors are employed which are not affected by the caustic and hydro treatment of the vat dye or where they can be resisted by the presence of oxidizing agents in the printing paste.

The cost of printing by this method is materially reduced since the color value obtained is considerably greater than the color value obtained in the conventional vat dye printing process, and the process permits higher productivity of the printing equipment.

Since the pastes contain no alkali or reducing agent, they may be stored for prolonged periods of time without deterioration.

The present invention also contemplates the preparation of novel printing compositions which are particularly applicable for use in the method of printing above described. The invention also contemplates the preparation of water-in-oil color concentrates containing the vat dye pigment in the aqueous phase in relatively high concentrations, which concentrates at the time of use can be diluted with a clear water-in-oil emulsion vehicle to give the desired concentration for the particular prints desired. The printing compositions of the present invention may be prepared from an aqueous dye paste which

is incorporated into a previously formed water-in-oil emulsion hereinafter referred to as the "W/O clear," or they may be produced from a previously prepared water-in-oil emulsion color concentrate in which the aqueous dye paste has been emulsified with a water-immiscible solvent together with dispersing agents and thickeners such as resins, etc.

The aqueous dye pastes which are usually incorporated in the water-in-oil emulsion to produce the emulsion printing pastes normally contain from 8% to 25% color solids and may contain from 1% to 10% of a dispersing agent or agents and other miscellaneous additives normally present in aqueous color printing pastes such as sodium acetate, sodium sulfate, carboxymethyl cellulose or other thickeners.

The water-in-oil emulsion color concentrates are usually prepared by homogenizing ordinary aqueous vat dye pastes into a colloidal dispersion or solution of resin in water-immiscible hydrocarbon solvents. These color concentrates will contain up to 25% color which is dispersed in the aqueous phase. In general these color concentrates will contain from 25 to 50 parts (by weight) of the oil phase which contains from 1.8 to 6.0 parts of resin, from 0 to 12 parts of pine oil or turpentine, the balance being a water-immiscible solvent such as "Varsol" No. 2; and from 75 to 50 parts of the oil phase which in turn contains from 5 to 25 parts of vat dye (dry basis) and from 0 to 6 parts of a dispersing agent, the balance being water.

The W/O clear will usually consist of from 20% to 35% of a hydrocarbon solvent such as "Varsol No. 2," or similar solvent to which is added from 2 to 7 parts by weight of an alkyd or other type resin dissolved in an aromatic hydrocarbon such as xylene, giving an actual resin concentration in the solution of from 1.2% to 4.2%, and from 58% to 78% by weight of water. Mixed hydrocarbon solvents of course may be employed, and other water-immiscible solvents such as turpentine, pine oil, etc., may be added to confer desirable characteristics to the printing paste. It is usually desired to add a small amount of an alkali metal carbonate to neutralize any acidity that may be present. Usually the addition of small amounts of neutral salts such as sodium chloride will increase the viscosity of the emulsion. The W/O clear emulsion should have a viscosity of between 300 and 39,000 centipoises as determined at 75° F.  $\pm 5^\circ$  in the Brookfield viscosimeter, using a No. 4 spindle at 12 r.p.m. If this paste is too viscous or too fluid, printable pastes are difficult to obtain when the aqueous dye paste or the water-in-oil emulsion color concentrate is added. It will be obvious to those skilled in the art that in the preparation of the W/O clear the emulsification should be carried out to a point where the dispersed phase is in very minute droplets, preferably below 5 microns.

The resins employed are preferably those which are self-emulsifying in the organic solvent with water, although emulsifying agents may be employed particularly with those which are otherwise difficult to emulsify in the system. The preferred resins are also those which are readily permeated or dissolved by the caustic alkali reducing solution so as to permit rapid reduction of the vat dye color prints.

The preferred class of resins for use in the preparation of these water-in-oil emulsion pastes are the alkyd resins, preferably the modified alkyd resins, which for the purpose of this invention are soluble in aqueous alkaline reducing solutions at 212° F. As examples of this type of resin, mention may be made of the Rohm & Haas "Duraplex A-27," which is an alkyd resin made by using approximately 42% phthalic anhydride and 37% cotton seed oil, the balance being the conventional polyhydric alcohol such as glycerin, glycol, etc., or those resins modified with other oils such as soya bean oil, etc., as further

illustrated in the examples. Usually these resins will be incorporated in the form of an organic solvent solution, since they are usually soluble in organic solvents and particularly in aromatic hydrocarbon solvents. Other resins such as the epoxy resins, melamine-formaldehyde resins, ureaformaldehyde resins, methacrylate resins, and the styrene-modified alkyd resins are illustrative of the types that may be employed, although, as stated above, the alkyd resins are preferred. Where resins are employed which are difficult to emulsify, it is usually advantageous to use small amounts of the alkyd resins as emulsifying agents. Other emulsifying agents, however, may be employed with these resins, such as esters of fatty acids, for example, lauric, palmitic or stearic acid esters of sorbitan and other alcohols, diethylaminoethylmethacrylate polymers, or copolymers of diethylaminoethylmethacrylate with fatty alcohol methacrylates such as "Lorol" methacrylate.

The organic water-immiscible solvent forming the oil phase of the water-in-oil emulsion paste (either color concentrate or W/O clear) should be one having a kauri-butanol value of from 40 to 100 so that the resin will have the desired degree of solubility in this oil. The preferred oils are those which have a high flash point, to reduce hazards in the printing process, and should be readily removable by washing or volatilized during the drying operation. The preferred class of organic solvents is the hydrocarbon solvents of the aliphatic, naphthenic and aromatic series, or mixtures of the same.

The water-in-oil emulsion (W/O clear) may be prepared by first emulsifying the liquid organic solvent containing the alkyd or other resin with water, and then adding to this emulsion the aqueous dye paste under high speed agitation or by merely mixing a color concentrate with the W/O clear with normal agitation. In this case, further emulsification is not required, which obviates the need for high speed homogenizing equipment.

Improved stability of the water-in-oil emulsion printing paste may be obtained by adding basic nitrogen-containing copolymer dispersing agents of the type described in U.S. Patent 2,737,452 of Catlin and Robbins in conjunction with other types of dispersing agents that may be normally used in standard aqueous printing pastes, preferably of the anionic type such as the naphthalene sulfonic acid-formaldehyde condensation products, or the ethylene oxide condensation products of arylalkyl phenols.

The water-in-oil emulsion printing pastes of the present invention will usually have the following general composition:

|                         | Percent        |
|-------------------------|----------------|
| Vat dye (dry)           | 0.02 to 6.0    |
| Resin                   | 1.0 to 4.5     |
| Total dispersing agents | 0.00015 to 3.0 |
| Total organic solvent   | 20.0 to 35.0   |
| Water                   | 78.98 to 51.5  |

In the above formula it is to be understood that when the basic nitrogen-containing dispersing agent above mentioned is used in the printing paste, it should not be to an extent greater than 0.8% when the maximum amount of dye is employed. The organic solvent employed is preferably of the aliphatic type, although it may contain high percentages of naphthenics and/or aromatics. Aromatic solvents such as solvent naphtha, xylene, and other water-immiscible phase.

The viscosity of the final water-in-oil emulsion printing paste can be varied by the addition of water or solvent to suit the particular printing conditions such as the type of design and engravings of the rollers or plates from which the design is printed.

It has now been found that the aqueous phase in the printing pastes of the present invention, which carries the insoluble vat dye, should be dispersed to the extent that the globules should have a maximum particle size

of 25 microns. It is preferred, however, that the aqueous droplets in the emulsion should not be greater than 16 microns.

The vat dye pastes used in the following examples are commercial standard vat dye pastes which contain from 0.075% to 1.5% of the dispersing agent generally referred to as the naphthalene sulfonic acid-formaldehyde condensation product or "Leucanol."

The following examples are given to illustrate the invention, it being understood that the invention is not limited thereto. The parts used are by weight, unless otherwise specified.

*Example 1*

(a) Three (3) parts of a xylene solution of a cotton seed oil modified alkyd resin (60% resin solids) of the type currently sold by Rohm & Haas under the designation "Duraplex A-27" is colloidally dispersed in 32 parts of a liquid hydrocarbon having a kauri-butanol value of 43.5, available on the market as "Varsol No. 2." This dispersion is emulsified with 65 parts of water, using a high speed homogenizer such as the Eppenbach mixer. The water-in-oil emulsion thus obtained has a viscosity of 1000 centipoises at 77° F. when determined in a Brookfield viscosimeter, Model LVF, employing a No. 4 spindle at 12 r.p.m. This emulsion is a light-colored, viscous paste. The alkyd resin employed in this example is made using 42% phthalic anhydride, 37% cotton seed oil, the balance being the conventional polyhydric alcohol such as glycerin, glycol, etc. As a 60% solution in xylene, this solution has a Gardner-Holdt viscosity rating of Z-7 and an acid number (of the solids) of 5-10.

(b) Ten (10) parts of a vat dye paste containing 19 weight percent color solids of a vat dye having Prototype No. 522 (as indicated in AATTC Technical Manual, 1955) is added to 90 parts of emulsion (a), using a high-speed mechanical homogenizer. The stable emulsion which is obtained is the printing paste.

(c) The printing paste of (b) is printed on cotton muslin fabric from an engraved copper roller. The printed fabric is then dried on hot cans for 1 to 5 minutes at from 220° to 275° F. The color-fugitive print is then developed by padding with an alkaline reducing solution which contains 4% by weight of caustic (sodium hydroxide), 6% by weight of sodium hydrosulfite, 0.1% by weight of a high fatty alcohol sodium sulfate surface-active agent having a chain of from 8 to 10 carbon atoms, and about 1% by weight of alkali-compatible starch. Within a fraction of a second, the fabric is passed through the above chemical-pad liquor and squeeze rolls, and then directly into an air-free steamer. During the 7 to 30 seconds that the fabric is in the steamer at from 214° to 290° F., the vat dye is reduced to its leuco form and fixed in the fiber. The prints are then finished by oxidizing the leuco form to the final insoluble vat dye by passing the fabric through 2% by weight of a hydrogen peroxide solution which is 16.5% by weight active oxygen, and 2% by weight of glacial acetic acid at 140° F. for 1 minute. The printed fabric is then scoured in 0.5% by weight of sodium oleate solution at 180° F. for 10 minutes, rinsed with clear water, and dried.

The tinctorial value of the resulting navy blue print as observed visually is equal to that obtained on application of a conventional aqueous paste (starch-sodium alginate thickener) containing 13.3 parts of the previously mentioned vat dye paste (Prototype No. 522) per 100 parts printing paste. Fastness to all common color-destroying agents, such as light, washing and crocking, is equal or superior to the fastness obtained with the aqueous color pastes.

*Example 2*

When 10 parts of the following vat dye pastes are used in the emulsion and the process described in Example 1, the tinctorial value of the resulting prints as above observed visually is equal to that obtained on application

of a conventional aqueous paste (starch-sodium alginate thickener) containing greater than 10 parts of the same dye paste per 100 parts of printing paste. Fastness to all common color-destroying agents, such as light, washing and crocking, is equal or superior to the fastness obtained with the aqueous color paste.

| Dye Paste (10 parts) | Colour Index No. | Percent Color Solids | Tinctorial Equivalent, Parts Dye Paste in Conventional Aqueous System |
|----------------------|------------------|----------------------|-----------------------------------------------------------------------|
| Jade Green.....      | 1101             | 11.2                 | 12.5                                                                  |
| Green.....           | PR 293           | 10.8                 | 13.3                                                                  |
| Yellow.....          | PR 9             | 9.8                  | 13.3                                                                  |
| Pink.....            | PR 109           | 14.6                 | 14.3                                                                  |
| Orange.....          | 1217             | 12.0                 | 15.4                                                                  |

*Example 3*

An emulsion is prepared as described in Example 1, except that 2 parts of turpentine is added to an alkyd resin (3 parts)-liquid hydrocarbon (30 parts) dispersion. The resulting emulsion has a viscosity of 1440 centipoises at 78° F. as determined in the viscosimeter described in Example 1.

When 10 parts of the following vat dye pastes are incorporated with 90 parts of the above emulsion and the printing process described in Example 1(c) is carried out, the tinctorial value of the resulting prints as observed visually is equal to that obtained on application of a conventional aqueous paste containing greater than 10 parts of the same dye paste per 100 parts of printing paste. Fastness to all common color-destroying agents, such as light, washing and crocking, is equal to or superior to the fastness obtained with the aqueous color paste.

| Dye Paste      | Colour Index No. | Percent Color Solids | Tinctorial Equivalent, Parts Dye Paste in Conventional Aqueous System |
|----------------|------------------|----------------------|-----------------------------------------------------------------------|
| Navy Blue..... | PR 522           | 19                   | 14.3                                                                  |
| Green.....     | PR 293           | 10.8                 | 51.3                                                                  |

*Example 4*

An emulsion is prepared as described in Example 1, except that 2 parts of pine oil is added to an alkyd resin (3 parts)-liquid hydrocarbon (30 parts) dispersion as used in Example 1. The resulting emulsion has a viscosity of 1400 centipoises at 77° F. as determined in the viscosimeter described in Example 1.

When 10 parts of the following vat dye pastes are incorporated with 90 parts of the above emulsion and the printing process described in Example 1 is carried out, the tinctorial value of the resulting prints as observed visually is equal to that obtained on application of a conventional aqueous paste containing greater than 10 parts of the same dye paste per 100 parts of printing paste. Fastness to all common color-destroying agents, such as light, washing and crocking, is equal or superior to the fastness obtained with the aqueous color paste.

| Dye Paste       | Colour Index No. | Percent Color Solids | Tinctorial Equivalent, Parts Dye Paste in Conventional Aqueous System |
|-----------------|------------------|----------------------|-----------------------------------------------------------------------|
| Green.....      | PR 293           | 10.8                 | 15.4                                                                  |
| Jade Green..... | 1101             | 11.2                 | 14.3                                                                  |
| Blue.....       | 1109             | 6.8                  | 12.5                                                                  |

*Example 5*

Three (3) parts of soya bean oil modified alkyd resin (a 60% resin solids in xylene reaction product of soya bean oil and phthalic anhydride in such proportions that

the complex reaction product contains 43% of chemically combined soya bean oil and the equivalent of 52% of glycerol phthalate and unreacted hydroxyl groups equivalent to 5% of glycerin) having a Gardner-Holdt viscosity rating of Y-Z1 and the resin solids of which has an acid number of 5-9, is colloidally dispersed in 30 parts of a liquid hydrocarbon having a kauri-butanol value of 43.5 ("Varsol" No. 2) and 2 parts of turpentine. The dispersion is emulsified with 65 parts of water by high speed agitation such as obtained with an Eppenbach mixer. The resulting water-in-oil emulsion has a viscosity of 440 centipoises at 77° F. as determined in the viscosimeter described in Example 1. When 10 parts of a vat dye paste containing 11.2% by weight color solids of Jade Green (Colour Index 1101) is incorporated with 90 parts of the above identified alkyd resin-hydrocarbon emulsion and printed as described under the procedure given in Example 1(c), the tintorial value of the resulting Jade Green print as observed visually is equal to that obtained on application of a conventional aqueous paste containing 11.8 parts of the same dye paste per 100 parts of printing paste. Fastness to all common color-destroying agents, such as light, washing and crocking, is equal or superior to the fastness obtained with the aqueous color paste.

*Example 6*

An emulsion is prepared as described in Example 1, except that 9 parts of the alkyd resin (60% solids) are employed together with 24 parts of the liquid hydrocarbon and 2 parts of turpentine. When emulsified as in Example 1, this gives a clear emulsion having a viscosity of 400 centipoises at 77° F.

When 10 parts of a standard commercial vat dye paste of an orange dyestuff, PR 381, containing 10.4 parts color solids, is emulsified with 90 parts of the above emulsion and the resulting water-in-oil emulsion is printed on cotton muslin fabric and developed in accordance with the procedure outlined in Example 1, clear, sharp prints are obtained which exhibit fastness properties equal to or greater than the same vat color when printed by conventional aqueous paste printing methods.

*Example 7*

A W/O clear emulsion is prepared according to Example 1 paragraph (a), substituting for the 32 parts of the particular liquid hydrocarbon 30 parts of solvent naphtha having a kauri-butanol value of 95, and 2 parts of turpentine. The resulting emulsion has a viscosity of 340 centipoises at 76° F.

When 10 parts of a standard commercial vat dye paste of the green dye of Colour Index 1101 containing 11.2% solids is emulsified with 90 parts of the above W/O clear, a stable water-in-oil emulsion printing paste is obtained which, when printed and developed by the process of Example 1 on spun rayon fabric, filament rayon fabric, mercerized broadcloth and dobby drapery fabric, gives prints of excellent fastness properties, sharpness of design and smoothness comparable to the prints of the foregoing examples.

*Example 8*

(a) Three (3) parts of a xylene solution of a cotton seed oil modified alkyd resin (60% resin solids), as used in Example 1, is mixed with 2 parts of pine oil and is colloidally dispersed in 21 parts of the liquid hydrocarbon used in Example 1. This dispersion is emulsified with 65 parts of water, using an Eppenbach homogenizer. A viscous, water-in-oil emulsion is obtained.

(b) Eighty (80) parts of a 40% solution of a copolymer prepared by copolymerizing 90 parts of "Lorol" fatty alcohol methacrylate and 10 parts of diethylaminoethyl methacrylate dissolved in a light petroleum lubricating oil, are emulsified in 15 parts of water in the presence of 5 parts of an ethylene oxide condensation

product of an aralkyl phenol dispersing agent ("Igepal CA").

(c) 0.5 part of the oil-in-water dispersion (b) is added to an aqueous paste consisting of 8.746 parts of water and:

0.662 part of a Green dye, C.I. 1101  
0.216 part of a Green dye, PR 293  
0.176 part of a Yellow dye, PR 9

10 which has been prepared by mixing the necessary amounts of the standard commercial vat dye pastes. This dye concentrate is added during vigorous mixing to 69.7 parts of the W/O clear prepared in paragraph (a) above. A viscous, stable water-in-oil emulsion 15 printing paste is obtained.

The above printing paste is printed on 80 x 80 cotton print cloth from shallow intaglio engraved copper printing rollers in a conventional textile printing machine and dried on conventional drying equipment at about 20 250° F. Subsequently, the fabric is impregnated at an 85% liquid pick-up with a 5% caustic soda-5% sodium hydrosulfite solution contained in a conventional dye padder threaded to give a single dip and single nip. The fabric is then immediately led into an air-free steam 25 atmosphere at a temperature of 214° F. and steamed for 13 seconds, rinsed, oxidized and soaped in open width. An excellent sharp, smooth, fast green print is obtained.

Examples 9 to 13, inclusive, illustrate the preparation 30 of color concentrates which can be readily mixed with the W/O clears at the time of printing by the use of simple mechanical agitators, since the color concentrate and W/O clear are already in a highly emulsified state and can be easily mixed. It is of course understood that the final mixture may be further diluted with the solvent 35 under normal mixing conditions or with water under high speed homogenization.

The color concentrates which are pigmented water-in-oil emulsions contain preferably from 25% to 50% by 40 weight of the oil phase and 75% to 50% of the aqueous phase. The oil phase will usually contain from 1.8% to 6% of the alkyd or other resin and up to 12% of pine oil, the balance being the organic solvent. The aqueous phase will contain from 5% to 20% of vat dye 45 solids and up to 0.6% of a dispersing agent or mixture of dispersing agents such as the naphthalene sulfonic acid-formaldehyde sodium salt, sodium lignin sulfonate, or the nitrogen-containing copolymer dispersing agents described above.

*Example 9*

(a) 600 parts of a press cake containing 33.5% of the dye of Colour Index 1101 is pasted with 2.0 parts of soda ash and 148 parts of water in a Werner-Pfeiderer mill until smooth.

55 The resulting aqueous phase is homogenized into an oil phase consisting of 90 parts of "Duraplex" A-27 resin solution (60% solids), 60 parts of pine oil and 100 parts of "Varsol" No. 2, using a high speed homogenizer such as the Eppenbach homomixer. The resulting water-in-oil emulsion is a smooth paste and contains 20% vat dye solids. These are located in the aqueous phase, i.e., they do not flush into the oil phase.

(b) A concentrated unpigmented or clear emulsion is prepared by Eppenbach-homogenizing the solution of 5 60 g. soda ash and 20 g. common salt in 375 g. water into a mixture of 500 g. "Duraplex" A-27 resin solution and 100 g. pine oil.

(c) A smooth print paste is prepared by mixing 50 g. of the color concentrate described in paragraph (a) with 50 g. of the clear concentrate described in paragraph (b), 300 g. "Sunoco Spirits" hydrocarbon solvent and 600 g. of water.

The resulting printing paste is printed on cotton muslin fabric from an engraved copper roller by the method 75 described in paragraph (c) of Example 1. The tintorial

value of the resulting green print is equal to that obtained on similar application of an aqueous printing paste (starch-gum tragacanth thickener) containing 5.0% more vat dye solids of Colour Index 1101. Fastness to all common color-destroying agents of the emulsion print is equal or superior to that of the aqueous system print.

*Example 10*

500 grams of the vat dye paste of PR 381 containing 11.2% dye solids and 0.6% naphthalene sulfonic acid-formaldehyde sodium salt dispersing agent (dry basis) is pasted with 2 grams of soda ash and 98 grams of water by stirring manually. The resulting aqueous phase is homogenized, using the Eppenbach homomixer, into 400 grams of an oil phase consisting of 90 grams of "Duraplex" A-27 resin solution, 60 grams of pine oil and 250 grams of hydrocarbon solvent such as "Varsol" No. 2.

The resulting thick, smooth paste contains 5.6% vat dye solids. A smooth printing paste is prepared by mixing 50 grams of this color concentrate with 50 grams of the concentrated unpigmented emulsion described in paragraph (b) of Example 9, 300 grams of "Varsol" No. 2 hydrocarbon solvent ("Esso") and 600 grams of water. The resulting printing paste is printed on cotton muslin by the method described in paragraph (c) of Example 1. The tinctorial value of the orange print produced with this emulsion printing paste is equal to that obtained on application of a conventional aqueous paste (starch-gum tragacanth thickener) containing 15% more vat dye solids of PR 381; in shade it is noticeably brighter than the aqueous system print. Fastness of the two prints to all common color-destroying agencies is essentially equal.

*Example 11*

500 grams of vat dye paste containing 11.2% of vat dye of PR 381 and 0.6% of naphthalene sulfonic acid-formaldehyde sodium salt is pasted with 2.0 grams of soda ash.

The resulting dispersion is homogenized (using an Eppenbach homomixer) into an oil phase containing 90 grams of "Duraplex" A-27 resin solution, 60 grams of turpentine and 348 grams of hydrocarbon solvent such as "Varsol" No. 2.

The resulting smooth vat dye pigmented emulsion contains 5.6% vat dye solids located in the aqueous phase. It is converted to a printing paste by the method described in Example 10. Its tinctorial value is equal to that obtained using the emulsion printing paste of Example 10, that is equal to that obtained using the aqueous printing paste of 15% greater color solids. Fastness of the corresponding comparative prints is essentially equal.

*Example 12*

500 grams of the khaki dye paste, PR 122, containing approximately 22% vat dye solids, 0.9% naphthalene sulfonic acid-formaldehyde sodium salt, and 0.2% partially desulfonated sodium lignin sulfonate is suspended in 200 grams of water. This dispersion is added while mixing with an Eppenbach homogenizer to an oil phase consisting of 30 grams of "Duraplex" A-27 resin solution, 20 grams of pine oil and 250 grams of hydrocarbon solvent such as "Varsol" No. 2. Mixing is continued for approximately five minutes to form a stiff smooth paste that contains approximately 11.0% vat dye solids. The vat dye is still located in the aqueous phase after homogenization.

When this concentrated pigmented emulsion is converted to a printing paste in the manner employed in Example 10 and printed on cotton muslin by the method described in paragraph (c) of Example 1, it yields prints tinctorially equal to but sharper and better covered than those obtained from a conventional starch-gum tragacanth-thickened aqueous system of equal pigment concentration. The prints are equal in fastness.

*Example 13*

220 grams of the vat dye used in Example 12 is dispersed in 480 grams of water. While Eppenbach homogenizing, this dispersion is added to an oil phase containing 100 grams of "Duraplex" A-27 resin solution, 120 grams of pine oil and 80 grams of "Varsol" No. 2.

The resulting concentrated emulsion contains in the aqueous phase 4.8% vat dye solids on the weight of the total emulsion. A printing paste produced from this emulsion by the method described in Example 12 also yields prints which are equal in tinctorial strength and in fastness to, but sharper and better covered than, one prepared from a conventional starch-tragacanth-thickened aqueous system of equal pigment concentration.

The following examples illustrate the use of various types of resin as the temporary binder for the pigment.

*Example 14*

13.7 parts of a blended resin consisting of equal parts of:

(1) An unmodified liquid epoxy resin having a viscosity of 10,000 to 14,000 centipoises [Brookfield viscometer, 23° C. (73° F.)] and an epoxy value of >0.480 eq./100 g., e.g., "Araldite" Liquid Resin No. 6010 marketed by Ciba Company, Inc.;

(2) an unmodified liquid epoxy resin having a viscosity of 20,000 to 40,000 centipoises [Brookfield viscometer, 23° C. (73° F.)] and an epoxy value of 0.440-0.480 eq./100 g., e.g., "Araldite" Liquid Resin No. 6020, is mixed with 1.3 parts of a xylene solution of a cotton-seed oil-modified alkyd resin (60% resin solids) having a viscosity of 35,000 to 40,000 centipoises. The mixture is then dispersed in 12.5 parts of a liquid hydrocarbon having a kauri-butanol value of 97.9 available on the market as "Solvesso" xylol. This dispersion is emulsified using a high-speed mixer with 72.5 parts of water in which has been dissolved 2.0 g./l. common salt and 0.25 g./l. sodium carbonate. The water-in-oil emulsion thus obtained has a viscosity of 39,000 centipoises at 77° F. when determined with a Brookfield viscometer, Model LVF, employing a No. 4 spindle at 12 r.p.m. This emulsion is a white-colored, viscous paste.

Ten (10) parts of a commercial vat dye paste having 19.1% color solids of a vat dye having Colour Index 1113, is added to 90 parts of the above emulsion, using a high-speed mechanical homogenizer. The stable emulsion which is obtained is the printing paste.

This printing paste is printed, developed and finished on cotton muslin fabric by the process described in Example 1. The tinctorial value of the resulting bright blue print as observed visually, is equal to that obtained on application of a conventional aqueous paste (starch-sodium alginate thickener) containing 25 parts of the previously mentioned vat dye paste (C.I. 1113) per 100 parts of printing paste.

*Example 15*

Six (6) parts of a petroleum spirits solution of a styrene-modified alkyd resin (50% resin solids) of the type currently sold by American Cyanamid Company under the designation "Cycopol" S-101-1 is colloidally dispersed in 29.5 parts of a liquid hydrocarbon having a kauri-butanol value of 43.5 available on the market as "Varsol" No. 2. This dispersion is emulsified with 64.5 parts of aqueous solution containing 2.0 g./l. common salt and 0.25 g./l. sodium carbonate, using an Eppenbach homomixer. The water-in-oil emulsion thus obtained has a viscosity of 11,500 centipoises at 77° F. when determined with a Brookfield viscometer, Model LVF, employing a No. 4 spindle at 12 r.p.m. This emulsion is a light-colored, viscous paste. The alkyd resin employed in this example is a 50% solution in petroleum spirits, having a Gardner color value of 3-6 and a Gardner-Holdt viscosity rating of  $Z_1-Z_4$  at 77° F. (25° C.).

Ten (10) parts of a commercial vat dye paste having

11

19.1% color solids of a vat dye having Colour Index 1113 is added to 90 parts of the above emulsion, using a high-speed mechanical homogenizer. The stable emulsion which is obtained is the printing paste.

The tinctorial value of the resulting bright blue print as observed visually is equal to that obtained on application of a conventional aqueous paste (starch-sodium alginate thickener) containing 16.7 parts of the previously mentioned vat dye paste (C.I. 1113) per 100 parts of printing paste.

*Example 16*

Nine (9) parts of a 60:40 butanol:xylene solution of a melamine-formaldehyde resin (50% resin solids) of the type currently sold by American Cyanamid Company under the designation "Melmac" 245-8, is blended with 1 part of a xylene solution of a cottonseed oil modified alkyd resin (60% resin solids). The mixture is colloidal-dispersed in 20 parts of a liquid hydrocarbon having a kauri-butanol value of 43.5, available on the market as "Varsol" No. 2. This dispersion is emulsified, using a high-speed mixer with 70 parts of water in which has been dissolved 2.0 g./l. of common salt and 0.25 g./l. of sodium carbonate. The water-in-oil emulsion thus obtained has a viscosity of 34,000 centipoises at 77° F. when determined with a Brookfield viscometer, Model LVF, employing a No. 4 spindle at 12 r.p.m. The emulsion is a light-colored viscous paste. The melamine-formaldehyde resin employed is a 50% solution and has a Gardner-Holdt viscosity of L-0 at 77° F. (25° C.) and the solid resin has an acid number maximum 1.

Ten (10) parts of a vat dye paste containing 11% color solids of the vat dye of C.I. 1101 is added to 90 parts of the above emulsion, using a high-speed mechanical homogenizer. The stable emulsion which is obtained is the printing paste. The printing paste is printed, developed and finished on cotton muslin fabric by the process described in Example 1.

The tinctorial value of the resulting blue-green print, as observed visually, is equal to that obtained on similar application of a conventional aqueous paste (starch-sodium alginate thickener) containing 25 parts of the previously mentioned vat dye paste (C.I. 1101) per 100 parts of printing paste.

When the alkyd resin of this example is replaced by from 0.125 to 0.5 parts of diethylaminoethylmethacrylate per part of the melamine-formaldehyde resin, a satisfactory emulsion is produced and the same desirable tinctorial value of the color is obtained in printing by the same method. The diethylaminoethylmethacrylate in this case is used as the dispersing agent for the melamine-formaldehyde resin.

*Example 17*

7.5 parts of a 40% solution of a copolymer prepared by copolymerizing 90 parts of "Lorol" fatty alcohol methacrylate and 10 parts of diethylaminoethyl methacrylate dissolved in a light petroleum lubricating oil, is dispersed in 1. parts of a liquid hydrocarbon having a kauri-butanol value of 97.9, available on the market as "Solvesso" xylol, and 20.0 parts of a second liquid hydrocarbon having a kauri-butanol value of 43.5 available on the market as "Varsol" No. 2. This dispersion is emulsified with 71.0 parts of water in which has been dissolved 2.0 g./l. of common salt, 2.0 g./l. of sodium sorbitol borate and 0.25 g./l. of sodium carbonate, using a high-speed mixer such as the Eppenbach mixer. The water-in-oil emulsion thus obtained has a viscosity of 1000 centipoises at 77° F. when determined in a Brookfield viscometer, Model LVF, employing a No. 4 spindle at 12 r.p.m. This emulsion is a light-colored viscous paste.

Ten (10) parts of a commercial vat dye paste of the blue dye C.I. 1113 is added to 90 parts of the above emulsion, using a high speed mechanical homogenizer. The stable emulsion which is obtained is the printing paste.

12

The above printing paste is printed, developed and finished on cotton muslin fabric by the process described in Example 1, giving a tinctorial value of the resulting blue print as observed visually, equal to that obtained on similar application of a conventional aqueous paste (starch-sodium alginate thickener) containing 20 parts of the same dye paste per 100 parts of printing paste.

The printing compositions and processes of printing of this invention may be employed in the printing of any cellulosic textile material or other textiles which can normally be dyed with vat dyes in the customary manner, namely, those which are not deleteriously affected by caustic alkalies in the concentrations and at the temperatures employed in the development of the vat dye.

The water-in-oil emulsion printing pastes of the present invention may be applied to textile materials from engraved rolls, plates, or by screen printing techniques. The application may be in patterns of single or multiple colors, overall application to solid shades, and either on one or both sides of the fabrics.

I claim:

1. In the process for printing textile materials with vat dyes in which the vat dye is subsequently developed with caustic alkali and an alkali metal hydrosulfite, the steps which comprise printing the vat dye on the textile material in the form of a water and oil emulsion in which the vat dye pigment is dispersed in a water phase and the oil phase contains from 1.0% to 4.5% of a caustic alkali-permeable resin of the group consisting of oil modified alkyd resins, epoxy resins, melamine formaldehyde resins, urea formaldehyde resins, methacrylate resins, and styrene-modified alkyd resins, the total amount of organic solvent in the emulsion comprising from 20.0% to 35.0%, the amount of water in the total amount comprising from 78.98% to 51.5% and the amount of dye present on a dry basis being from 0.02% to 6.0%, the organic solvent of the emulsion being one that has a kauri-butanol value of from 40 to 100, drying the material so printed, padding the dried material with an aqueous solution of a reducing agent consisting of caustic alkali and sodium hydrosulfite, steaming the material so padded in air-free steam at temperatures of from 212° F. to 290° F. for a period of from 7 to 30 seconds, oxidizing the reduced vat dye on the textile material, washing and drying.

2. The process of claim 1 in which the alkali-permeable resin is a drying oil-modified alkyd resin.

3. The process of claim 1 in which the alkali-permeable resin is a cottonseed oil-modified alkyd resin.

4. A water-in-oil dye emulsion for use in vat dye printing consisting essentially of from 25 to 50 parts of an oil phase consisting of an organic water-immiscible solvent having a kauri-butanol value of from 40 to 100 and from 75 to 50 parts of a water phase, the oil phase containing from 1.8 to 6.0 parts of a caustic hydrosulfite-permeable resin of the group consisting of oil modified alkyd resins, epoxy resins, melamine formaldehyde resins, urea formaldehyde resins, methacrylate resins, and styrene-modified alkyd resins, from 0 to 12 parts of a solvent of the group consisting of pine oil and turpentine, and the balance being a water-immiscible solvent; the aqueous phase containing from 5 to 25 parts of vat dye (dry basis) and from 0 to 6 parts of a dispensing agent, the balance being water.

5. A printing paste for use in the coloring of textile materials which may be applied from intaglio rolls of a conventional textile printing machine, consisting essentially of a water-in-oil emulsion in which a vat dye is dispersed in the oil phase consisting of an organic water-immiscible solvent having a kauri-butanol value of from 40 to 100 and a caustic hydrosulfite-permeable alkyd resin is present in the oil phase, said printing paste having the general composition as follows: 0.02% to 6.0% of vat dye (dry), 1.0% to 4.5% of caustic hydrosulfite-permeable alkyd resin, 0.00015% to 3.0% of total dis-

65  
50  
40  
35  
25  
10  
70  
75

13

persing agents, 20.0% to 35.0% total organic solvent, and from 78.98% to 51.5% of water.

6. A printing paste for use in the coloring of textile materials which may be applied from intaglio rolls of a conventional textile printing machine, prepared by incorporating an aqueous vat dye paste containing a small amount of a water-soluble dispersing agent in an oil emulsion containing a caustic hydrosulfite-permeable alkyd resin, which oil emulsion contains from 20% to 35% of a hydrocarbon solvent having a kauri-butanol value of from 40 to 95, from 58% to 78% by weight of water and from 1.2% to 4.2% by weight of an alkyd resin, and a small amount of an oil-soluble dispersing agent, said oil emulsion prior to the addition of the dye paste

10

14

having a viscosity of from 300 to 39,000 centipoises at 75° F.  $\pm 5^\circ$ , the said printing paste having the water droplets in the water-in-oil emulsion of a size not greater than 25 microns.

5. The product of claim 6 in which the water droplets in the water-in-oil emulsion are of a size not greater than 16 microns.

## References Cited in the file of this patent

## UNITED STATES PATENTS

|           |            |               |
|-----------|------------|---------------|
| 2,288,261 | Abrams     | June 30, 1942 |
| 2,323,871 | Kienle     | July 6, 1943  |
| 2,587,905 | Saville    | Mar. 4, 1952  |
| 2,594,899 | Fordemwalt | Apr. 29, 1952 |

UNITED STATES PATENT OFFICE  
CERTIFICATE OF CORRECTION

Patent No. 2,907,624

October 6, 1959

Arthur K. Saville

It is hereby certified that error appears in the printed specification of the above numbered patent requiring correction and that the said Letters Patent should read as corrected below.

Column 3, line 46, for "75° F. + 5°" read — 75° F.  $\pm$  5° —; column 11, lines 23 and 24, for "obtained" read — obtained —; line 58, for "1. parts" read — 1.5 parts —; column 12, line 63, for "dispensing" read — dispersing —.

Signed and sealed this 12th day of April 1960.

(SEAL)

Attest:

KARL H. AXLINE  
Attesting Officer

ROBERT C. WATSON  
Commissioner of Patents